

## UNITED STATES PATENT OFFICE

2,124,055

## ABRASIVE ARTICLE

Robert P. Courtney, Maplewood, N. J., assignor to  
 Bakelite Corporation, New York, N. Y., a corporation of Delaware

No Drawing. Application May 18, 1934,  
 Serial No. 726,366

14 Claims. (Cl. 51—278)

This invention relates to abrasive articles, such as sandpaper and the like, and to a novel method for the production of such articles, and is particularly directed to a method and product involving an improved bonding medium for attaching abrasive grains to a fibrous base.

Varnishes composed of drying oils, raw or modified, with or without natural or synthetic resins, or of resins alone, dissolved in suitable solvents have heretofore been used as adhesives for bonding sand, grits, or other abrasive particles to fibrous bases such as paper, cloth, and the like.

There are several disadvantages involved in this procedure. If on drying or baking the varnish or adhesive becomes brittle it is essential that it should not penetrate too deeply into the fibrous base, else it will cause the fibrous base and the resulting abrasive article to be brittle and to lack strength and shock resistance. Even if the dried varnish is flexible it is desirable that the fibrous base should not be penetrated very deeply for reasons of economy in the use of the binding medium.

To reduce such penetration, varnish compositions of the type described above have been heated or otherwise treated so as to very substantially increase their "body" or viscosity. As a result they are sometimes difficult to manufacture due to the tendency of the varnish to become completely solid while bodying, before the heating or other treatment can be discontinued. For the same reason the keeping quality of such varnish compositions is often unsatisfactory. Varnishes of such high viscosity are frequently more difficult to handle in applying to the fibrous base than a less viscous liquid.

These viscous or heavy bodied varnish compositions have a decreased tendency to flow around the abrasive particles. It is largely upon this surrounding of the abrasive particle that the strength of adherence of the adhesive to the particle depends, so that the increasing of the viscosity of the varnishes entails a very decided disadvantage in lessened bonding strength as compared with the more fluent compositions.

I have found that if varnishes of the type described above, but having a relatively low viscosity, are emulsified in water or other non-solvent before applying to the fibrous base the following advantages are obtained:

If the non-solvent has a preferential ability to wet the fibrous backing, which is usually the case when water is used as a non-solvent medium, the backing will be first wetted by the non-solvent

and the varnish will remain on or near the surface. It will usually dry on the surface sufficiently to prevent material penetration before the non-solvent has evaporated from the fibrous base. The same varnish applied without emulsifying in a non-solvent will penetrate the fibrous base quite readily.

A varnish of low viscosity, when made into an emulsion and applied to a fibrous base, will surround abrasive particles subsequently placed upon the wet surface more readily and fix them more strongly than the same varnish treated to give a higher viscosity.

Such emulsions of low viscosity varnishes are more easily manufactured, keep better, and are more easily applied to the fibrous base than the same varnish made to a higher viscosity.

A substantial saving is effected in quantities used, due to lowered penetration. Moreover, such emulsions, if of the oil-in-water type, or, more exactly, varnish in non-solvent, can be thinned with the non-solvent. Many non-solvents, especially water, are cheaper than solvents for these materials.

It is advantageous to control the conditions under which the emulsion of the varnish composition is made so as to favor the dispersion of the varnish in the water or other non-solvent. It is possible, however, to have the water in the disperse phase in a varnish medium provided the conditions of use are such that when the emulsion is applied to a fibrous base the water particles contact the base and there is a preferential absorption of the water particles by the base.

As an illustration of a varnish emulsion suitable for use in the present invention, an oil-resin composition is prepared in accordance with the disclosure of U. S. Patent 1,677,417 to Turkington, from cresol, formaldehyde, tung oil, and some rosin with hexamethylene tetramine as a converting agent. A suitable solvent, such, for example, as a mixture of xylol and butyl acetate is added to form a varnish. An emulsifying agent, for example, triethanolamine is also preferably added. In general, the amount of triethanolamine or other emulsifying agent added to the oil-resin composition is advantageously about 2 to 10% of the water used in forming the emulsion. The varnish thus prepared is then gradually added to the water with agitation to form an emulsion. Pigments, colors, or other addition agents can be incorporated with the composition at this stage, if desired.

The amount of varnish that can be included in a given amount of water with the varnish re-

maining as the disperse phase depends upon the agent and speed of agitation; but as high as 99% of the emulsion can be varnish without changing over into a water-in-varnish emulsion as indicated 5 by tests made by diluting with water.

As an additional illustration of a suitable composition, an oil-soluble resin is prepared by reacting a phenyl-phenol compound with formaldehyde, preferably with the amount of formaldehyde in excess of molecular proportions, in the presence of a catalyst such as oxalic acid. This resin after dehydration is made into a varnish by heating with a fatty oil, for example, as tung oil; best results seem to follow from heating about 15 equal weights of resin and tung oil for about an hour at about 200° C. and then incorporating such additional amounts of tung oil or other fatty oil or mixture of tung oil and other fatty oil as linseed oil, as may be desired, followed by a 20 short heating period. For air-drying varnishes or coating compositions it is desirable to include a small percentage of a drier such as 0.1 to 1.0 per cent of cobalt linoleate or other known drying agent. Suitable solvents such as petroleum 25 solvents, cellosolve (monoethyl ether of glycol), xylol or mixtures of these are stirred into the mass while it is maintained at a suitable temperature; the amount of solvent added depends upon its insolubility in water and the viscosity desired, 30 but a weight of a water insoluble solvent as specified above equal to the weight of the oil-resin composition yields a varnish suitable for most purposes. To prepare an emulsion of such a varnish, casein, for example, is dispersed in 35 water made ammoniacal by the addition of strong ammonia; the varnish is slowly added into the casein solution and agitation causes an emulsion to form. The more rapid the agitation the thicker will be the emulsion. If the varnish is added too 40 rapidly, the emulsion may become one of water in varnish, but slow addition and rapid agitation produces a varnish in water emulsion. The nature of the emulsion is determined by adding a small amount to water; if it can be dispersed in 45 the water it is regarded as one of varnish in water. Varnish in water emulsions are preferred since the possibility of dilution with water permits the use of relatively small amounts of water-insoluble solvents in the preparation of the varnishes.

50 As emulsifying agents a wide variety of substances can be used. For example, gelatin, camphor, tannic acid, lamp black, lead acetate, starch, gum arabic, acid casein solution, soaps and the like normally produce emulsions of varnish 55 in water. Bentonite, ammonium linoleate, triethanolamine and its fatty acid soaps or compounds and basic casein solutions quite readily form emulsions of varnish in water; in general these are preferred agents. It is not necessary, 60 however, in every case that an emulsifying agent be included; some varnishes apparently have ingredients present that function as emulsifying agents.

In the preparation of abrasive articles, varnish 65 emulsions of the type described above are applied, for example by spreading rolls, upon a fibrous base, such as paper or cloth. The varnish component of the emulsion spreads out into a uniform film on the base, without substantially penetrating the base. When abrasive particles, such as sized sand grains, are spread upon the varnish film in accordance with the usual practice in the art, the particles are readily 70 wet and surrounded by the varnish film, which 75 upon hardening by air-drying or baking or the

like, provides a tough, strong bond for the abrasive particles.

The term varnishes is used herein as equivalent to the expression "coating compositions". These compositions are generally solutions; but it is 5 to be understood that oil-resin compositions in the liquid form not necessarily incorporating solvents and which can be applied in the same manner as varnishes to form coatings are comprehended within the meaning of the term 10 varnishes.

I claim:

1. A method of making abrasive articles which comprises coating a fibrous base with an emulsion of a penetrative varnish composition in a volatile 15 non-solvent liquid, applying abrasive particles to the varnish film thereby produced, and hardening the varnish film.

2. A method of making abrasive articles which comprises coating a fibrous base with an emulsion 20 of a penetrative varnish composition in water, applying abrasive particles to the varnish film thereby produced, and hardening the varnish film.

3. A method of making abrasive articles which comprises coating a fibrous base with an emulsion 25 of a penetrative varnish composition including a phenolic resin in a volatile non-solvent liquid, applying abrasive particles to the varnish film thereby produced, and hardening the varnish film.

4. A method of making abrasive articles which comprises coating a fibrous base with an emulsion of a penetrative varnish composition including a phenolic resin of the oil-soluble type in a volatile 35 non-solvent liquid, applying abrasive particles to the varnish film thereby produced, and hardening the varnish film.

5. A method of making abrasive articles which comprises coating a fibrous base with an emulsion of a penetrative varnish composition including a phenolic resin of the oil-soluble type in water, 40 applying abrasive particles to the varnish film thereby produced, and hardening the varnish film.

6. Method of making an abrasive article which comprises emulsifying a penetrative varnish composition in a non-solvent medium, coating a fibrous base with the emulsion, applying abrasive particles to the varnish film thereby produced, and hardening the varnish film.

7. Method of making an abrasive article which comprises emulsifying a penetrative varnish composition in water, coating a fibrous base with the emulsion, applying abrasive particles to the varnish film thereby produced, and hardening the varnish film.

8. Method of making an abrasive article which comprises emulsifying a penetrative varnish composition including an oil-soluble phenolic resin in water, coating a fibrous base with the emulsion, applying abrasive particles to the varnish film 60 thereby produced, and hardening the varnish film.

9. Abrasive article comprising a fibrous base, a binder consisting of a varnish composition inherently penetrative to said base forming a substantially non-penetrating uniform layer in direct contact with the surface of said base, and abrasive grains embedded in said varnish layer.

10. Abrasive article comprising a fibrous base, a binder consisting of an oil-resin varnish composition inherently penetrative to said base forming a substantially non-penetrating uniform layer in direct contact with the surface of said base, and abrasive grains embedded in said varnish layer.

11. Abrasive article comprising a fibrous base, a binder consisting of a phenolic resin varnish composition inherently penetrative to said base forming a substantially non-penetrating uniform layer in direct contact with the surface of said base, and abrasive grains embedded in said varnish layer.
12. Abrasive article comprising a fibrous base, a binder consisting of an oil-soluble phenolic resin varnish composition inherently penetrative to said base forming a substantially non-penetrating uniform layer in direct contact with the surface of said base, and abrasive grains embedded in said varnish layer.
13. Abrasive article comprising a paper base, a binder consisting of a varnish composition inherently penetrative to said base forming a substantially non-penetrating uniform layer in direct contact with the surface of said base, and abrasive grains embedded in said varnish layer.
14. Abrasive article comprising a fabric base, a binder consisting of a varnish composition inherently penetrative to said base forming a substantially non-penetrating uniform layer in direct contact with the surface of said base, and abrasive grains embedded in said varnish layer.

ROBERT P. COURTNEY.